

May 8, 1951

A. GLAZUNOV

2,552,423

PROCESS FOR THE DIRECT PRODUCTION OF REFINED ALUMINUM

Filed Nov. 30, 1948

FIG. 1



FIG. 2



INVENTOR.  
ALEXANDRE GLAZUNOV

BY

*A. Glazunov*

ATTORNEY

## UNITED STATES PATENT OFFICE

2,552,423

PROCESS FOR THE DIRECT PRODUCTION  
OF REFINED ALUMINUM

Alexandre Glazunov, Geneva, Switzerland

Application November 30, 1948, Serial No. 62,643  
In Switzerland November 30, 1947

1 Claim. (Cl. 204—67)

1

Alloys having the best properties are obtained, when produced from the purest metals. Industrial plants therefore demand the highest possible purity and the problem of refining is becoming more and more important.

Processes for refining aluminium have been known for a long time; among the chief methods employed is that of purification by means of electrolysis, in a furnace. This method is known as the "three layers refining."

The various furnaces employed for this procedure (Hoopes, Péchiney) differ only in the details of their construction; the procedure requires rather complicated and expensive manipulation, as well, as an addition of 30% copper, which increases the specific weight of the lower layer.

The present invention eliminates these difficulties and enables the purest aluminium to be obtained in one furnace, by means of a single operation, starting from  $Al_2O_3$ , without addition of copper, or any other manipulations.

The furnace consists of two containers, communicating at their bases, where two electrolyses may proceed simultaneously.

(a) The first electrolysis of  $Al_2O_3$  dissolved in cryolite and  $CaF_2$  (the usual electrolyte for this operation) produces crude aluminium.

(b) The second electrolysis refines this crude aluminium by means of the electrolyte usually employed in refining furnaces.

The crude liquid aluminium, obtained in the first electrolysis acts as a bipolar electrode, functioning simultaneously as cathode for the first and as an anode for the second electrolysis, since it flows between the two electrolytes.

The annexed drawing indicates one possible rendering of such a furnace, which could, of course, be modified to any appropriate form.

In the drawings:

Fig. 1 is a central vertical sectional view of a furnace embodying my invention; and

Fig. 2 is a plan view of the same.

As shown in the drawing the furnace indicated generally at P includes an outer container 1 preferably provided with a lining 2 of suitable refractory material, such as  $MgO$ , resistant to the corrosive action of the melted salts used for the electrolysis. If desired, the walls of this container may be provided with auxiliary electrodes for the initiation of the procedure within the furnace. As illustrated, the bottom of the container 1 may either be formed from refractory material, like the walls, or it may be partially or completely constructed of an auxiliary electrode, also intended for use in connection with the initiation of the procedure.

Within the outer container 1 is an inner container 4, open at the top and bottom, and spaced from the bottom of the outer container, thus

2

forming two compartments. Preferably the inner container is provided with a suitable lining 5, of graphite or the like, which terminates short of the lower extremity of said inner container.

Positive electrodes 6 are positioned within the inner container 4 so as to dip into or be immersed in the solution B of  $Al_2O_3$  in cryolite, an electrolyte normally used for the production of crude aluminium. The negative pole of this electrolysis is composed of melted crude aluminium, indicated at  $Al1$  beneath the solution B within the inner container.

The second electrolysis, effected by the electrolyte C which is of higher specific gravity than molten aluminium, has a soluble anode, comprising crude aluminium, as a positive pole and the negative pole comprises the layer of refined aluminium indicated at  $Al2$ , in contact with the negative electrodes 3 which are positioned in a zone located within the outer container 1, exteriorly of the inner container 4.

I claim:

15 An improvement in the process of producing refined aluminium, which comprises arranging a layer of aluminium refining electrolyte of higher specific gravity than molten aluminium below a layer of crude molten aluminium, placing a layer of aluminium producing electrolyte of lower specific gravity than molten aluminium on the upper surface of the crude aluminium, passing an electrolyzing current from a fixed anode through the aluminium producing electrolyte in contact therewith to the crude aluminium as a bipolar electrode and through the aluminium refining electrolyte to a fixed cathode in contact therewith, feeding  $Al_2O_3$  into said aluminium producing electrolyte, and collecting the refined molten aluminium formed at the cathode at a portion of the upper surface of the refining electrolyte which is in a zone electrically and physically separated from the fixed anode, the aluminium producing electrolyte and the crude aluminium layer.

45 ALEXANDRE GLAZUNOV.

## REFERENCES CITED

The following references are of record in the file of this patent:

## UNITED STATES PATENTS

| Number       | Name    | Date          |
|--------------|---------|---------------|
| 830,051      | Carrier | Sept. 4, 1906 |
| 1,833,425    | Jessup  | Nov. 5, 1931  |
| 55 1,937,509 | Burgess | Dec. 5, 1933  |

## FOREIGN PATENTS

| Number     | Country       | Date          |
|------------|---------------|---------------|
| 500,509    | Great Britain | Feb. 10, 1939 |
| 60 220,856 | Germany       | Apr. 8, 1910  |